

## UNITED STATES PATENT OFFICE

2,195,584

## DARK COLORED TEXTILE MATERIAL

George W. Seymour and Victor Sluyty Salvin,  
Cumberland, Md., assignors to Celanese Corporation of America, a corporation of Delaware

No Drawing. Application February 11, 1938,  
Serial No. 190,040

13 Claims. (Cl. 8—48)

This invention relates to the production of dark-colored textile materials that are made of or contain organic derivatives of cellulose and, more particularly, to the method of producing a black color in or on such textile materials.

An object of this invention is the economic and expeditious production of black-dyed fabrics and other textile materials made of or containing an organic derivative of cellulose, the coloration being effected by applying a diazotizable dyestuff base to the material, diazotizing and coupling with a naphthoic or similar acid. Another object of this invention is the production of black fabrics or other textile materials, made of or containing organic derivatives of cellulose, that do not crock or bleed and that are more fast to acid and light fading than fabrics dyed by methods employed prior to this invention. Other objects of our invention will appear from the following detailed description.

By employing this invention, there is effected an improvement both in reducing crocking and/or bleeding and a more uniform standard shade is obtained. In accordance with this invention, there are produced black fabrics containing organic derivative of cellulose yarns that do not bleed pink when rubbed with a similar but undyed fabric wet with perspiration nor crock black when rubbed with a dry white fabric. For the purpose of describing this invention the term "crocking" will be used as including bleeding or other forms of dyeing defects that allow the black fabric to color white fabric attached thereto when the two fabrics are washed, dry cleaned, subjected to perspiration, acid fumes or rubbing.

By employing this invention, there is also produced a black fabric containing organic derivative of cellulose yarns that is more fast to acid fading and light fading than similar black fabrics produced prior to this invention. The stability of the dyed fabric is extremely good making it exceptionally well suited as a lining fabric for coats or other wearing apparel.

It is known that there are three major forms of crocking of fabric containing organic derivatives of cellulose that are dyed black with diazotized dyestuffs. First, and least desirable, is a pink-to-red crocking which appears to vary in intensity with different batches of dyed fabric. The tendency of this type of pink-to-red crocking is to bleed off from a coat lining fabric when wet with perspiration. Crocking in another form is evidenced as a black coloration which also appears to vary in intensity with different batches, with different qualities of fabric and with the same quality of fabric which has been processed in two batches by apparently identical means. The third form of crocking appears as an oily black substance which is readily removable by thorough scouring, which scouring, however, is sometimes required to be more severe than fabrics containing organic derivatives of cellulose can withstand. We have found that by employing this invention, these types of crocking can be eliminated or substantially eliminated without the addition of costly reagents or additional processing steps. At the same time a more stable fabric is produced that has a faster color.

In accordance with this invention, we apply a diazotizable black dye base to a fabric containing an organic derivative of cellulose, the fabric is then treated in a bath containing hydrochloric acid (or other suitable mineral acid) to form the dihydrochloride completely and then diazotize the base in the presence of a still further amount of mineral acid. The acid bath preceding the diazotizing bath becomes slightly colored showing the removal of superficial dye base and metallic impurities of the dyestuff. The bath may contain about 5 ccs. of acid per liter, say from 3 ccs. to 10 ccs. per liter. The mineral acid must be removed prior to coupling, preferably by washing. We have found that this washing should be carried out with as little exposure of the diazotized fabric as possible to light, heat and air. To reduce the time employed in washing free of acid we prefer to employ a washing bath containing sodium acetate, sodium carbonate or other soluble neutralizing salts. When sodium acetate is employed in the bath, better shades are obtained and pink-to-red crocking is substantially eliminated. After washing to remove excess acid and the salts formed in neutralizing the acid, the fabric is coupled with a suitable coupling compound, preferably  $\beta$ -oxy-naphthoic acid. In order to decrease the decomposition products caused by side reactions in the coupling process, the diazotized fabric must be coupled soon after diazotization has been completed. The temperature and pH value of the coupling bath must be closely controlled while the accessibility of the coupling compound to the fabric and the thorough adsorption of the coupling compound into the fabric must be observed. The coupling operation should be performed by running the fabric two or three ends at 20° C. in a jig or its equivalent on a winch to promote efficient adsorption and then 1 to 3 ends at 38° C. to 42° C. to promote coupling with a final end at about 60° C. to 75° C. to accelerate coupling and to decompose any remaining azo group. The coupling compound is dispersed in the treating bath with the aid of dispersing agents with sufficient buffer salts (preferably sodium acetate or sodium bicarbonate) to maintain the pH value of the bath at between 5 and 7. The coupling compound couples best at about a pH value of 7 or higher, but then it is present as a metallic salt which is not readily adsorbed by the fabric.

Therefore, the pH value should be 7 or slightly below, preferably between 5 and 7.

This invention is applicable to yarns, fibers, ribbons, straws, etc., but more especially to fabrics made of or containing organic derivatives of cellulose such as the organic esters of cellulose and the cellulose ethers. Examples of the organic esters of cellulose are cellulose acetate, cellulose formate, cellulose propionate and cellulose butyrate, while examples of the cellulose ethers are ethyl cellulose, methyl cellulose and benzyl cellulose.

The fabric to be treated may be made wholly of organic derivative of cellulose material or it may contain other materials such as cotton, silk, wool and the like. The fabric may be woven, knitted, netted, knotted, etc., and may be in the form of taffetas, crepes, nimon, voile, velvets or the like. The textile material may also be formed into an article prior to imparting color thereto, i. e., stockings, men's hose, gloves, underwear, etc.

The dye base to be applied to the textile material may be aniline-4-azo-4- $\alpha$ -naphthylamine or analogues of the same which when coupled with a suitable coupling agent produces a dark color. Suitable analogues and the color they produce when coupled with  $\beta$ -oxy-naphthoic acid are phenol-4-azo-4- $\alpha$ -naphthylamine (bluish black), benzene-azo-4- $\alpha$ -naphthylamine (reddish black), para-methoxy-benzene-azo-4- $\alpha$ -naphthylamine (bluish black of very good depth), ortho - methoxy-benzene-azo-4- $\alpha$ -naphthylamine (purplish black) and naphthalene-azo-4- $\alpha$ -naphthylamine (slightly reddish black).

The coupling compound is preferably  $\beta$ -oxy-naphthoic acid or its analogues which produces a black or substantially black color on the fabric. However, the invention is also applicable where coupling compounds that produce a blue color or a red color or combinations of these colors are employed. Examples of such coupling compounds are  $\alpha$ -naphthol,  $\beta$ -naphthol, phenol, salicylic acid and their derivatives or substitution products.

It has been customary in the past to apply the dye base to the fabric and then diazotize in a bath containing a nitrite and a mixture of formic, hydrochloric and/or sulphuric acids. We have found that a more uniform shade and a reduced amount of crocking is produced when only inorganic acids are employed in the diazotizing bath and when the dihydrochloride of the dye base is preformed in the fabric prior to the application of the diazotizing bath. The use of only mineral acids and the preformation of the mineral acid salts of the dye base in the fabric produces a fabric having a diazotized dye base therein that is relatively stable up to about 60° C. Thus the fabric can be washed free of acid and placed in the coupling bath without decomposition products being formed. However, washing of the diazotized fabric should be done briefly, with cold water and shielded from the light and air. Washing causes hydrolysis of the diazonium salt as; diazonium sulphate  $\rightarrow$  diazonium hydrate  $\rightarrow$  diazo hydrate. Both hydrates are less stable than the diazonium salt. Also, when sufficient mineral acid is used diazotization is between 90% and 100% complete, provided, however, that there is an excess of the mineral acid employed. For instance, when diazotizing aniline 4-azo-4- $\alpha$ -naphthylamine 11 mols of the dye base are employed, and 42 mols of sodium nitrite and 44 mols of hydrochloric acid or its

equivalent are the absolute minimum necessary for complete diazotization. For improved results to be derived in accordance with this invention the presence of an excess of mineral acid is required. This excess should be about  $\frac{1}{2}$  mol of acid per amino group and this excess is made up of the total acid used in preforming the mineral acid salt of the dye base and a quantity of acid added to the diazotizing bath. The excess acid, however, may be from about  $\frac{1}{2}$  mol to 1 mol excess of acid per amino group to be diazotized. Due to the excess acid present during the diazotization step it is preferable to maintain the temperature at between 5 to 10° C. with ice or artificial cooling means to prevent injury to the dyestuff, fabric or machine and to the operator due to the evolution of acid fumes. Preformation of the amino salt is used in part to insure a large excess of mineral acid without increasing the concentration of acid in the diazotization bath. Thus the presence of  $\text{HNO}_2$  in the atmosphere about the jig is avoided. Nitrous acid is not only obnoxious to the operators but may have harmful effects upon shades being dyed on adjacent machines.

After diazotization it is necessary to subject the fabric to a washing process in order to remove the excess inorganic acid. This is necessary for two major reasons, one to prevent the precipitation of the coupling compound as a non-reactive material and, second, to enable the coupling to proceed thoroughly and uniformly. The diazotized fabric must be washed thoroughly, and quickly without exposure to air, light or heat. Exposure of the fabric produces an irreversible decomposition of the diazonium compound which, after it occurs, greatly increases the tendency of the dyed fabric to crock. The amount of dye base applied to the fabric may be any suitable amount, say from 0.1 to 6% by weight of the fabric.

After the dye base has been applied to the fabric, diazotized and the fabric washed free of excess mineral acid, the fabric is subjected to an operation including the application thereto of a coupling compound under such conditions that the coupling compound reacts with the diazonium compound formed from the dye base. The coupling reaction must always be looked upon as a race between azo compound formation and decomposition of the diazonium compound. Some diazonium compounds are so sensitive to this factor that rigid control of the pH value of the treating bath is necessary to obtain consistent results in the dyeing of textiles. In this respect the dyeing of textiles containing organic derivatives of cellulose are different from other textile materials as the organic derivative of cellulose textile materials do not readily adsorb the salts of the coupling compound. Therefore, in order to have the coupling compound satisfactorily adsorbed on the fibers it must be present as an acid rather than its salt. Obviously, therefore, the pH value of the aqueous dispersion of the coupling compound must be below 7, preferably between 5 and 7, as below this point an adsorption readily takes place but coupling is sluggish and acid reaction compounds are formed.

In the coupling operation the temperature of the treating bath must also be controlled in order to produce an improved dyeing and a uniform shade from batch to batch. In order to decrease the decomposition products from side

reactions to the coupling process the diazotized fabric must be subjected to the coupling reagent immediately after diazotization has been completed. The temperature of the bath at the time the fabric is subjected thereto is preferably around 20° C. for at this temperature the adsorption of the coupling compound by the fabric is greatly facilitated. The temperature should then be raised to about 40° C. to promote coupling and retard decomposition, blackening of the fabric, due to coupling, does not occur until this temperature has been reached. The temperature should then be rapidly raised to above 60° C., preferably between 60 and 75° C., to accelerate coupling and to decompose the remaining azo groups. For instance, when dyeing the fabric on a jig the fabric is run two ends at 20° C. to permit thorough incorporation of the  $\beta$ -oxy-naphthoic acid in the fiber, two ends at 40° C. for at this temperature coupling starts, then two ends at 70° C. in order to complete the coupling of the sluggish reaction. The high temperature should be avoided initially since decomposition of the diazonium compound of the dye base is accelerated at those temperatures.

The bath from which the coupling compound is applied to the fabric is preferably formed by dispersing the coupling compound in a dispersing agent approaching neutrality and well buffered with such salts as sodium acetate or sodium bicarbonate for changes in pH value. It is known that if the particle size of the coupling compound is controlled by the use of a dispersing agent a great reduction in the amount of crocking of the dyed fabric is obtained. The use of the dispersing agent is imperative also in that it controls the particle size and disperses the coupling materials which form the coupling bath, thus making a more uniform and thorough penetration of the coupling compound into the fabric. This dispersion also prevents the superficial formation of the dye on the outside of the fabric and also to the deposition of non-dispersible compounds adhering to the fabric from the coupling process. Obviously the dispersing agent should have no reaction with the coupling compound. Suitable dispersing mediums which may be employed with the coupling compounds listed above are a mixture of Turkey red oil and xylol, the sodium salt of sulphated lauryl alcohol or other higher fatty alcohol, sulphonated vegetable oils, dextrin, sulphated naphthene and similar dispersing mediums or mixtures of the same.

In order to further illustrate our invention, but without being limited thereto, the following example is given:

#### EXAMPLE

##### Rinse

2 ends cold; 2 ends at 90° C.—to set the fabric to the jig.

##### Basing

|                                            |        |         |
|--------------------------------------------|--------|---------|
| Fabric                                     | grams  | 150,000 |
| Water                                      | liters | 500     |
| Black dyebase                              | grams  | 2,900   |
| 70 Sulphonated naphthalene ricinoleic acid | do     | 2,600   |
| Gardinol                                   | do     | 3,000   |
| Soda ash                                   | do     | 800     |
| Temperature, 90° C.; time, 50 ends=1000    |        |         |
| 75 min.                                    |        |         |

**Scouring**

|                                             |        |       |
|---------------------------------------------|--------|-------|
| Gardinol                                    | grams  | 3,000 |
| Soda ash                                    | do     | 800   |
| Water                                       | liters | 500   |
| Temperature, 90° C.; time, 10 ends=200 min. |        | 5     |

**Pre-formation of the salt**

|                                       |        |         |
|---------------------------------------|--------|---------|
| Water                                 | liters | 500     |
| 33% HCl                               | do     | 2.5-2.7 |
| Or 95% H <sub>2</sub> SO <sub>4</sub> | do     | 1.3-1.5 |
| Temp. 18-25° C.; time, 2 ends=40 min. |        | 10      |

**Diazotization**

|                                                                                                                                   |        |       |
|-----------------------------------------------------------------------------------------------------------------------------------|--------|-------|
| Water                                                                                                                             | liters | 500   |
| Sodium nitrite                                                                                                                    | grams  | 3,500 |
| H <sub>2</sub> SO <sub>4</sub> (1/2 previous quantity, however, the HCl formed in the previous step maintains the desired excess) | ccs    | 1,000 |
| Temp. 18-22° C.; time, 3-4 ends=60-80 min.                                                                                        |        | 20    |

**Wash**

|                                                      |        |     |
|------------------------------------------------------|--------|-----|
| Cold water                                           | liters | 500 |
| (Sodium acetate optional)                            | grams  | 500 |
| (Residual HNO <sub>2</sub> or HCl negligible.)       |        |     |
| Temperature, 18-20° C.; time, 2 to 3 ends=40-60 min. |        | 25  |

**Coupling**

|                                                                                                 |        |        |
|-------------------------------------------------------------------------------------------------|--------|--------|
| Water                                                                                           | liters | 500    |
| $\beta$ -oxy-naphthoic acid                                                                     | grams  | 3,000  |
| Celascour                                                                                       | do     | 61,000 |
| Gardinol                                                                                        | do     | 6,100  |
| Temperature: 4 ends at 18-25° C.=80 min.; 2 ends at 40° C.=40 min.; 4 ends at 60-70° C.=80 min. |        | 35     |

This bath should have a pH of 6-6.5 and should not change materially during processing.

##### Wash

Washing may be carried out with either hot or cold water in order to free the fabric from the ingredients of the coupling bath.

With regard to the amount of water retained in the fabric before, between and after each processing step, the fabric is at all times thoroughly wetted out after the initial step of setting to the jig. The amount of water retained by the fabric will probably be between two and five times the weight of the fabric, depending upon the type of fabric, weave, twist, and whether or not it was mixed with cotton, viscose, silk, etc.

The fabric after drying is found to be colored a good black and to be exceptionally fast to light and acid-alkali or perspiration fading. The chemical stability of the organic derivative of cellulose in the fabric is found to be substantially as good as the stability of the undyed material.

It is to be understood that the foregoing detailed description is merely given by way of illustration and that many variations may be made therein without departing from the spirit of our invention.

Having described our invention, what we desire to secure by Letters Patent is:

1. Process for the production of dark colored textile materials containing an organic derivative of cellulose by a process employing diazotizable dyestuffs, which comprises applying a diazotizable dyestuff base to said textile material, applying a mineral acid to said textile material to form therein the mineral acid salt of the dyestuff base, diazotizing and coupling with a coupling component producing a dark color.

2. Process for the production of dark colored textile materials containing cellulose acetate by a process employing diazotizable dyestuffs, which comprises applying a diazotizable dyestuff base to said textile material, applying a mineral acid to said textile material to form therein the mineral acid salt of the dyestuff base, diazotizing and coupling with a coupling component producing a dark color. 5
10. 3. Process for the production of dark colored textile materials containing an organic derivative of cellulose by a process employing diazotizable dyestuffs, which comprises applying a diazotizable dyestuff base to said textile materials, applying hydrochloric acid to said textile material to form therein the dihydrochloride salt of the dyestuff base, diazotizing and coupling with a coupling component producing a dark color. 10
15. 4. Process for the production of dark colored textile materials containing cellulose acetate by a process employing diazotizable dyestuffs, which comprises applying a diazotizable dyestuff base to said textile materials, applying hydrochloric acid to said textile material to form therein the dihydrochloride salt of the dyestuff base, diazotizing and coupling with a coupling component producing a dark color. 15
20. 5. Process for the production of dark colored textile materials containing cellulose acetate by a process employing diazotizable dyestuffs, which comprises applying a diazotizable dyestuff base to said textile material, applying a mineral acid to said textile material to form therein the mineral acid salt of the dyestuff base, diazotizing, 25 washing free of excess acid while the textile material is secluded from light, heat and air and coupling with a coupling component producing a dark color. 25
30. 6. Process for the production of dark colored textile materials containing cellulose acetate by a process employing diazotizable dyestuffs, which comprises applying a diazotizable dyestuff base to said textile material, applying a mineral acid to said textile material to form therein the mineral acid salt of the dyestuff base, diazotizing, 35 washing free of excess acid while the textile material is secluded from light, heat and air and coupling with a coupling component producing a dark color. 35
40. 7. Process for the production of dark colored textile materials containing cellulose acetate by a process employing diazotizable dyestuffs, which comprises applying a diazotizable dyestuff base to said textile material; applying a mineral acid to said textile material to form therein the mineral acid salt of the dyestuff base, diazotizing and applying to the textile material a dispersion of a coupling component producing a dark color dispersed in water with the aid of a dispersing medium. 45
50. 8. Process for the production of dark colored textile materials containing cellulose acetate by a process employing diazotizable dyestuffs, which comprises applying a diazotizable dyestuff base to said textile material, applying a mineral acid to said textile material to form therein the mineral acid salt of the dyestuff base, diazotizing and applying to the textile material a dispersion of a coupling component producing a dark color dispersed in water with the aid of a dispersing medium while maintaining the pH value of the coupling bath between 5 and 7. 50
55. 9. Process for the production of dark colored textile material to form therein the mineral acid salt of the dyestuff base, diazotizing and applying to the textile material a dispersion of a coupling component producing a dark color dispersed in water with the aid of a dispersing medium while maintaining the pH value of the coupling bath between 5 and 7 with the aid of basic salts. 5
10. 10. Process for the production of dark colored textile materials containing cellulose acetate by a process employing diazotizable dyestuffs, which comprises applying a diazotizable dyestuff base to said textile material, applying a mineral acid to said textile material to form therein the mineral acid salt of the dyestuff base, diazotizing, 15 washing the textile material in a bath containing basic salts and coupling with a coupling component producing a dark color. 15
15. 11. Process for the production of dark colored textile materials containing cellulose acetate by a process employing diazotizable dyestuffs, which comprises applying an amino azo compound to said textile materials, treating said textile materials with a mineral acid, in a quantity at least equivalent to the amino azo compound incorporated in said textile materials, to form therein the mineral acid salt of the amino azo compound, diazotizing and coupling with a coupling component producing a dark color. 20
20. 12. Process for the production of dark colored textile materials containing cellulose acetate by a process employing diazotizable dyestuffs, which comprises applying an amino azo compound to said textile materials, treating said textile materials with hydrochloric acid, in a quantity at least equivalent to the amino azo compound incorporated in said textile materials, to form therein the dihydrochloride salt of the amino azo compound, diazotizing and coupling with  $\beta$ -oxy-naphthoic acid. 25
25. 13. Process for the production of dark colored textile materials containing cellulose acetate by a process employing diazotizable dyestuffs, which comprises applying aniline-4-azo-4- $\alpha$ -naphthylamine to said textile materials, 30 treating said textile materials with hydrochloric acid, in a quantity at least equivalent to the aniline-4-azo-4- $\alpha$ -naphthylamine incorporated in said textile materials, to form therein the dihydrochloride salt of the aniline-4-azo-4- $\alpha$ -naphthylamine, diazotizing and coupling with  $\beta$ -oxy-naphthoic acid. 35
30. 14. Process for the production of dark colored textile materials containing an organic derivative of cellulose by a process employing diazotizable dyestuffs, which comprises applying aniline-4-azo-4- $\alpha$ -naphthylamine to said textile materials, 40 treating said textile materials with hydrochloric acid, in a quantity at least equivalent to the aniline-4-azo-4- $\alpha$ -naphthylamine incorporated in said textile materials, to form therein the dihydrochloride salt of the aniline-4-azo-4- $\alpha$ -naphthylamine, diazotizing and coupling with  $\beta$ -oxy-naphthoic acid. 45
35. 15. Process for the production of dark colored textile materials containing cellulose acetate by a process employing diazotizable dyestuffs, which comprises applying aniline-4-azo-4- $\alpha$ -naphthylamine to said textile materials, treating said textile materials with hydrochloric acid, in a quantity at least equivalent to the aniline-4-azo-4- $\alpha$ -naphthylamine incorporated in said textile materials, to form therein the dihydrochloride salt of the aniline-4-azo-4- $\alpha$ -naphthylamine, diazotizing and coupling with  $\beta$ -oxy-naphthoic acid. 50
40. 16. Process for the production of dark colored textile materials containing cellulose acetate by a process employing diazotizable dyestuffs, which comprises applying aniline-4-azo-4- $\alpha$ -naphthylamine to said textile materials, treating said textile materials with hydrochloric acid, in a quantity at least equivalent to the aniline-4-azo-4- $\alpha$ -naphthylamine incorporated in said textile materials, to form therein the dihydrochloride salt of the aniline-4-azo-4- $\alpha$ -naphthylamine, diazotizing and coupling with  $\beta$ -oxy-naphthoic acid. 55
45. 17. Process for the production of dark colored textile materials containing cellulose acetate by a process employing diazotizable dyestuffs, which comprises applying aniline-4-azo-4- $\alpha$ -naphthylamine to said textile materials, treating said textile materials with hydrochloric acid, in a quantity at least equivalent to the aniline-4-azo-4- $\alpha$ -naphthylamine incorporated in said textile materials, to form therein the dihydrochloride salt of the aniline-4-azo-4- $\alpha$ -naphthylamine, diazotizing and coupling with  $\beta$ -oxy-naphthoic acid. 60

GEORGE W. SEYMOUR.  
VICTOR SLUYTY SALVIN.